

March 8, 1932.

W. A. WISSLER

1,848,289

METHOD OF WELDING COMPOSITE ARTICLES

Filed July 7, 1928



Fig. 1.



Fig. 2.

INVENTOR:

William A. Wissler,  
BY  
Byers, Townsend & Bickenstein  
ATTORNEYS.

## UNITED STATES PATENT OFFICE

WILLIAM A. WISSLER, OF JACKSON HEIGHTS, NEW YORK, ASSIGNOR TO HAYNES STELLITE COMPANY, A CORPORATION OF INDIANA

## METHOD OF WELDING COMPOSITE ARTICLES

Application filed July 7, 1928. Serial No. 291,006.

My invention relates to methods of making composite articles consisting of a foundation metal and a shield or surface layer of metal deposited on the foundation in a fused condition.

Machine tools, for example, are made in this way by depositing high speed steel or stellite on the tip or cutting portion of a steel shank by means of an oxy-acetylene torch or an 10 electric arc. A deposit of metal of sufficient thickness is usually formed to permit regrinding and sharpening of the tool. Sometimes a notch or a depression is formed in which metal is deposited. Other articles such as 15 railway rail members are shielded or armored by depositing stellite on the parts that are subjected to wear.

In forming the deposit the foundation metal becomes highly heated to a considerable 20 depth, often to a red heat, and as a result the fused metal cools and solidifies slowly in its interior and in portions which are in contact with the foundation metal. The result is that the portion of the deposited metal exposed to the air is the first to solidify. When 25 the fused metal is completely solidified, a shrinkage pocket or porous spot occurs in the portion in which solidification is delayed.

It is among the objects of my invention to 30 provide methods and means of depositing such fused-on shields without producing an unsound portion within the body of the deposited metal.

I have found that if the foundation metal 35 is cooled so that the solidification of the fused-on metal will occur progressively from the surface of the foundation metal toward the surface of the fused-on metal, the porous portion will either not be formed or will be so 40 close to the surface that a light grinding will remove it. One method of cooling the foundation metal consists in partially submerging the metal in a cooling bath of water or other liquid, in such a manner that the portion upon 45 which the fusion heat is directed will project

above the surface of the bath. Such an arrangement will effect the desired cooling of the foundation metal and prevent the formation of a pipe in the fused-on metal.

A more practical device which I have used is shown in a side elevational view in Fig. 1 and in Fig. 2 in a view in cross-section taken along the line II—II of Fig. 1. Cooling members 1 are held by any convenient means, such as the clamps 2 in contact with the foundation metal 3. The cooling members 1 are provided with guards of heat insulating material 4 which may be strips of asbestos. These members protect the members 1 from the intense heat used to fuse the shielding metal. 50 The members 1 may be solid blocks of metal, for example, copper, but I prefer to provide channels 5 through which a cooling fluid may be supplied at the desired rate from a suitable source through the pipes 6 and discharged 55 through the pipes 7. For the best results the cooling members 1 are preferably shaped to conform to the surface of the foundation member. The surface upon which the metal is deposited is generally located a short distance above the surface of the cooling members. This distance may be regulated according to the rate at which heat is supplied to the metal and the rapidity with which the cooling members conduct away the heat. 60 Heat should not be extracted from the foundation metal rapidly enough to prevent the deposited metal from forming a strong bond 65 with the foundation metal, but there should be enough cooling to cause a progressive solidification from the surface of the foundation metal as the fused metal is deposited and to prevent an accumulation of fused metal in the interior of the deposit 8. The cooling 70 may also be regulated by increasing or decreasing the flow of cooling fluid through the channels 5.

I claim as my invention:

Process of building up a composite métal article consisting of a body of foundation 80

metal and a surface layer of metal more wear-resistant than said foundation metal, which comprises contacting the said body with cooling members in such manner that a portion of the body protrudes a regulatable distance beyond said cooling members and depositing on said protruding portion a layer of the surfacing metal by means of a gas welding flame, the extent of protrusion of said portion being so regulated as to produce progressive solidification of the deposited metal from the surface of said body.

In testimony whereof, I affix my signature.

WILLIAM A. WISSLER.

15

20

25

30

35

40

45

50